

Dec. 28, 1948.

J. H. HUNTER

2,457,154

PHONOGRAPH RECORD

Filed July 26, 1941

THIN PLAYING SURFACE OF AN AGGREGATE INCLUDING A  
BINDER AND FILLERS AND HAVING LOW "SURFACE NOISE"  
CHARACTERISTIC.



RELATIVELY THICK CORE PROVIDING OVER-ALL  
MECHANICAL PROPERTIES OF THE PRESSED RECORD.

INVENTOR

James H. Hunter

BY

Lennie, Davis, Marin and Edmonds  
ATTORNEYS

## UNITED STATES PATENT OFFICE

2,457,154

## PHONOGRAPH RECORD

James H. Hunter, Bridgeport, Conn., assignor to  
Columbia Records Inc., a corporation of Delaware

Application July 26, 1941, Serial No. 404,204

5 Claims. (Cl. 154—43)

1

This invention relates to a phonograph record of the laminated type and it has for its objects the provision of a record relatively economical to manufacture having a playing surface of low "surface noise" characteristic and of good wearing quality under constant use.

The above objects are attained, according to the present invention, by providing a relatively thick core adapted to substantially determine the over-all mechanical properties of the record after pressing, and a thin playing surface of an aggregate including a binder and a first comminuted filler material having irregular particles varying in size from substantially less than a micron up to the order of four microns in largest dimension, and a second finely-divided filler material having substantially uniform size particles of an order permitting ready dispersion thereof both upon the surfaces of and between the irregular size particles. The ratio of binder to the total amount of said fillers is such that, after pressing, the particles of the fillers are homogeneously distributed in close relation substantially without intervals therebetween.

As the result of extensive investigation, it has been found, contrary to the description of United States Patent No. 2,221,270, that the use of fillers having substantially uniform size particles of the order therein described, yield what will be termed a brittle playing surface having a high "surface noise" characteristic. By the use of an aggregate including a binder as above described, comparable to concrete aggregate, i. e., different size stones, sand, and cement, a playing surface having a very low surface noise is obtained which stands up under constant wear better than the playing surfaces heretofore proposed. In addition, it has been found that a playing surface in the form of an aggregate including a binder in accordance with the invention, wears the point of the reproducing needle less than any shellac type record now upon the market. This may be attributed to the fact that the particles of the fillers used in the improved compound and aggregate are so minute that they produce very little grinding action on the needle point.

Since surface noise is the audible result of the grinding action of the fillers on the needle point, it may be reduced by reduction in the effective particle size of the fillers. In reducing the effective particle size of the fillers, it was found that needles lasted longer, indicating less wear of the playing surface.

The art of molding and pressing phonograph records of the laminated type is well understood.

2

When manufacturing the improved records in accordance with the present invention in the form of single or double face disc records, paper sheets coated with the playing surface material may be used on one or both sides of the core material, as the case may be. In the record pressing operation carried out with the customary press, the relatively thick core serves as a mechanical support for the thin playing surface or surfaces.

Core material suitable for use in accordance with the invention is composed essentially, for example, of green slate filler, cotton flock, and a binder such as shellac or resin or both. Since the core material is employed solely for the purpose of producing a relatively thick core to provide support for the thin playing surface or surfaces, and to establish the over-all mechanical properties of the record, its constituents may be varied, as will be readily understood. Anyone of the well-known compositions for core material may be employed for the purposes of the invention.

The following example illustrates a preferred formula for the aggregate including the binder, to be used for the thin playing surface, parts being given by weight:

|                    |     |
|--------------------|-----|
| Diatomaceous earth | 165 |
| Tibar HH           | 228 |
| Carbon black       | 39  |
| Shellac            | 145 |
| Calcium stearate   | 1/4 |

It will be observed that the shellac binder constitutes approximately 25% by weight of the aggregate. Thus, the ratio of binder to filler is substantially one to three.

After thorough mixing of the above constituents, the powdered material is appropriately applied to discs of paper of suitable size for forming the playing surface of the records.

The diatomaceous earth is comminuted by fine grinding to produce irregular particles varying in size from substantially less than a micron up to three or four microns in largest dimension. As is well known, this material is porous in structure.

The constituent Tibar HH is a precipitated pigment of titanium dioxide and barium sulfate. The nature of the chemical precipitation is such that the particles are of substantially uniform size and of the order of one-quarter micron.

Due to the small particle size of the Tibar HH, it is readily dispersed into the pores and upon the surfaces of the diatomaceous earth particles.

The amount of shellac or binder employed and the ratio thereof to filler (diatomaceous earth and Tibar HH) is such that, after pressing, the

particles of said fillers are homogeneously distributed in close relation substantially without intervals therebetween.

Other materials may be substituted for the material Tibar HH, for example titanium dioxide per se or any other of the known precipitated and extremely fine fillers and the like. Also mixtures of shellac and other natural and synthetic resins may be employed, such as the natural resins congo gum and manila gum and the synthetic resins, for example, poly-vinyl acetate and its various derivatives.

A cross-sectional view of a laminated sound record made in accordance with the present invention is shown in the accompanying drawing.

It is to be understood that the foregoing description of a preferred embodiment is set forth by way of example or illustration and that the thin playing surface of an aggregate including a binder may be composed of various ingredients and produced in various ways for the particular purpose for which it is required and that the invention is not limited to these specific embodiments, except as defined in the accompanying claims.

I claim:

1. A laminated sound record comprising a relatively thick core adapted to substantially provide the over-all mechanical properties of the pressed record, and a thin playing surface of an aggregate including a binder and a first filler of comminuted diatomaceous earth having irregular particles varying in size from substantially less than a micron up to the order of four microns in largest dimension, and a second filler having substantially uniform size particles of the order of one-quarter micron permitting ready dispersion thereof both upon the surfaces of and between said diatomaceous earth particles, the ratio of binder to filler being of the order of one to three so that after pressing the particles of said fillers are homogeneously distributed in close relation substantially without intervals therebetween.

2. A laminated sound record comprising a relatively thick core adapted to substantially provide the over-all mechanical properties of the pressed record, and a thin playing surface of an aggregate including a binder and a first filler of comminuted diatomaceous earth having irregular particles varying in size from substantially less than a micron up to the order of four microns in largest dimension, and a second chemically precipitated filler of titanium dioxide and barium sulfate having substantially uniform size particles of the order of one-quarter micron permitting ready dispersion thereof both upon the surfaces of and between said diatomaceous earth particles, the particles of said fillers being, after pressing, homogeneously distributed in close relation substantially without intervals therebetween.

3. A laminated sound record comprising a relatively thick core adapted to substantially provide the over-all mechanical properties of the pressed record, and a thin playing surface of an aggregate including a shellac binder and a first filler of comminuted diatomaceous earth having irregular

particles varying in size from substantially less than a micron up to the order of four microns in largest dimension, and a second chemically precipitated filler of titanium dioxide and barium sulfate having substantially uniform size particles of the order of one-quarter micron permitting ready dispersion thereof both upon the surfaces of and between said diatomaceous earth particles, the particles of said fillers being, after pressing, homogeneously distributed in close relation substantially without intervals therebetween.

4. A laminated sound record comprising a relatively thick core adapted to substantially provide the over-all mechanical properties of the pressed record, and a thin playing surface of an aggregate including a binder and a first filler of comminuted diatomaceous earth having irregular particles varying in size from substantially less than a micron up to the order of four microns in largest dimension, and a second filler comprising titanium dioxide and having substantially uniform size particles of the order of one-quarter micron permitting ready dispersion thereof both upon the surfaces of and between said diatomaceous earth particles, the ratio of binder to filler being of the order of one to three so that after pressing the particles of said fillers are homogeneously distributed in close relation substantially without intervals therebetween.

5. A laminated sound record comprising a relatively thick core adapted to substantially provide the over-all mechanical properties of the pressed record, and a thin playing surface of an aggregate including a binder and a first filler of comminuted diatomaceous earth having irregular particles varying in size from substantially less than a micron up to the order of four microns in largest dimension, and a second filler of chemically precipitated fine material having substantially uniform size particles of the order of one-quarter micron permitting ready dispersion thereof both upon the surfaces of and between said diatomaceous earth particles, the ratio of binder to filler being of the order of one to three so that after pressing the particles of said fillers are homogeneously distributed in close relation substantially without intervals therebetween.

JAMES H. HUNTER.

#### REFERENCES CITED

The following references are of record in the file of this patent:

#### UNITED STATES PATENTS

| Number    | Name           | Date           |
|-----------|----------------|----------------|
| 1,207,383 | Edison         | Dec. 5, 1916   |
| 1,623,285 | Stone          | Apr. 5, 1927   |
| 1,919,920 | Whyte          | July 25, 1933  |
| 1,926,130 | Whyte          | Sept. 12, 1933 |
| 1,997,398 | Whyte          | Apr. 9, 1935   |
| 2,006,378 | Redhill et al. | July 2, 1935   |
| 2,130,239 | Hunter         | Sept. 13, 1938 |
| 2,206,636 | Hunter         | July 2, 1940   |
| 2,216,970 | Walker         | Oct. 8, 1940   |
| 2,217,170 | Hunter         | Oct. 8, 1940   |
| 2,221,270 | Severin        | Nov. 12, 1940  |